

March 5, 1929.

H. M. NAUGLE ET AL

1,704,015

## CONTINUOUS ANNEALING AND CLEANING PROCESS

Filed July 1, 1925

2 Sheets-Sheet 1



### Inventors

*H. M. Naugle and  
A. J. Townsend*

By Grease and Bond  
Attorneys

March 5, 1929.

H. M. NAUGLE ET AL

1,704,015

CONTINUOUS ANNEALING AND CLEANING PROCESS

Filed July 1, 1925

2 Sheets-Sheet 2

Fig. 2



Inventors

H. M. Naugle and  
A. J. Townsend

By *Frease and Bond*

Attorneys

## UNITED STATES PATENT OFFICE.

HARRY M. NAUGLE AND ARTHUR J. TOWNSEND, OF CANTON, OHIO, ASSIGNEES, BY  
MESNE ASSIGNMENTS, TO THE COLUMBIA STEEL COMPANY, OF PITTSBURGH, PENN-  
SYLVANIA, A CORPORATION OF PENNSYLVANIA.

## CONTINUOUS ANNEALING AND CLEANING PROCESS.

Application filed July 1, 1925. Serial No. 40,739.

The invention relates to a continuous method for quickly annealing a strip of sheet metal, referred to in a general way in our application for method of making strip sheets, 5 filed August 22, 1922, Serial No. 583,612, matured in Letters Patent No. 1,536,028, issued April 28, 1925, and reissued June 14, 1927, as No. 16,652; and this application is a continuation of the common subject matter in 10 our pending application filed November 17, 1924, Serial No. 750,271 for the same invention.

The general object of the improvement is to anneal the metal in a manner that will give 15 the product the uniform ductile and other structural characteristics which are necessary for deep drawing and forming or stamping operations.

We have discovered that slow or continued 20 heating of steel sheet metal induces a grain growth therein, and that a continued maintenance at and above scaling temperature fosters the formation of scale on the surface thereof.

25 The grain growth resulting from a slow or continued heating of sheet steel is increased in metal which has been critically strained as by being rolled previous to the heating and especially so in low carbon steels.

30 The formation of scale which is induced by a continued maintenance of the metal at and above the scaling temperature is a chemical reaction between gas in the air and the steel itself; and no doubt, like most chemical 35 reactions the speed at which the action takes place increases as the temperature of the steel increases, and the formation may begin actively on low carbon steel heated in the air at about 1150° F.

40 Furthermore the formation of scale on the surface of steel sheets is more or less irregular, and the pickling required to remove the same must be of sufficient strength and duration to remove the heaviest deposit of scale, 45 during which time the steel surface is unevenly attacked by the pickling solution, which produces an uneven surface on the steel after the scale has been removed.

A complete readjustment of the grains of 50 the metal to relieve them of the strains produced by a rolling operation, and more particularly by a rapid cold rolling reduction and other reductions forming like strains, cannot be accomplished by the ordinary box

annealing of a mass or coil of metal, for the 55 reason that the longer period of time required for properly heating the inner portions of the mass or coil, not only results in the over-annealing of the outer portion thereof, but in the production of a grain growth 60 in a considerable portion of the mass or coil, which destroys the ductility and uniformity, and also decreases the strength of the material in the outer portions of the mass or coil.

The present improvement is particularly 65 concerned with the annealing of steel having a carbon content of less than .20%, for the reason that such a low carbon steel is best suited for deep drawing and forming or stamping operations; and for properly annealing the same, the metal must be uniformly heated to a temperature of from 1300° to 70 1600° F. As a grain growth, sometimes known as "Stead's brittleness", may occur at 75 a temperature less than 1300° F., if the same is maintained long enough; one object of the present improvement is to uniformly heat the metal quickly to an annealing temperature, to maintain or continue that temperature only long enough, say about one minute, 80 to correct the micro-structure of the steel which has been critically stressed by previous rolling processes while avoiding any material grain growth, and then to promptly cool the metal quickly and uniformly, without, however, quenching the same to harden its structure.

The general object of the improvement 85 may be attained by annealing a strip, a sheet, or other thin flat stock, by the direct action of 90 electric resistors, while moving continuously through a heating chamber, in which the resistors are transversely located adjacent to and parallel with the strip, by which the same may be uniformly heated and the degree 95 of heat definitely controlled at all points in the heating furnace; and then to promptly and quickly cool the strip by moving it continuously through a tubular duct surrounded by a moving body of water or other heat absorbing liquid, by which the strip may be 100 quickly and gradually reduced to a non-oxidizing temperature when exposed to the air.

A further object of the present improvement is to avoid or overcome difficulties which 105 may accompany the continuous annealing process set forth in our application for patent, filed April 4, 1924, Serial No. 704,157,

and the use of the continuous annealing apparatus set forth in our application for patent filed herewith, Serial No. 750,269; in both of which an effort is made to carry on the 5 heating and cooling operations in the presence of a neutral or reducing gas, to the exclusion of air, for preventing or removing an oxidation or discoloration of the surface of the strip.

- 10 The very desirable and highly efficient use of electric resistors for directly heating a strip of steel or the like for annealing the same in a chamber containing a reducing gas, requires the use of a refractory lining for 15 the heating chamber and preferably requires the use of a liquid seal for the opening through which the strip enters the chamber. It has been found, however, that the use of a deoxidizing medium in the heating chamber 20 has an injurious effect upon the electric resistors, and the vapors resulting from the volatilization of a liquid sealing medium has a deteriorating effect upon the refractory lining.
- 25 And a particular object of the present improvement is to avoid or overcome the difficulty which may accompany the continuous annealing and cleaning processes set forth in our application for patent filed herewith, 30 Serial No. 750,270, in which a heat retaining deoxidizing duct is interposed between the heating chamber and the cooling duct for cleaning the strip from oxidation and discoloration before it is cooled.
- 35 The use of such a heat retaining deoxidizing duct may sometimes maintain the metal at an annealing temperature for such an extended period, as will result in an incipient or a substantial grain growth; and in any 40 event the chemical reaction which results in the elimination of surface oxidation gives two products, one of which is gaseous and the other solid; and the solid product is deposited on the strip in the form of a fine dust, so 45 that when the strip sheet is subsequently handled or processed this dust cracks and results in what is known as "surface breaks".

The present improvement avoids these difficulties by the use of an unsealed heating 50 chamber and cooling duct in which some atmospheric gas may enter and slightly oxidize or discolor the surface of the strip, but does not form a scale which cannot be removed by a continuous cleaning in a weak acid solution; 55 and by providing, in series, a cleaning tank and a washing tank immediately in rear of the cooling duct, for removing any oxidation or discoloration there may be on the strip when it leaves the cooling duct, and completely 60 cleaning the strip with a smooth finish without leaving any deposits thereon.

By these means the detrimental effect upon the refractory lining of the heating chamber by the volatilization therein by a liquid seal- 65 ing medium, and the damaging action of a

reducing gas upon the electric resistors within the heating chamber, are both avoided; and the cooling of the strip is effected so promptly and quickly after it is annealed that no opportunity is given for any objectionable 70 grain growth, and the strip is subsequently subjected to the cleaning and washing operations, so that upon the completion of the processes, the body of the strip is uniformly ductile and the surface is clean and smooth. 75

The improved method may be carried out by the apparatus illustrated, more or less conventionally, in the accompanying drawing forming part hereof, in which—

Figure 1 is a side elevation, partly in section of the apparatus; and

Fig. 2, a diagram showing the heat curve of the metal during the improved process.

Similar numerals refer to similar parts throughout the drawing.

The apparatus may include a coil box A, a strip leveler B, a traveling spot welder C, a solution washer D, an electric heating furnace E, a cooling duct F, a pickling tank G, a washing tank H, conveyer rolls I, a double 90 end shear J and a strip coiler K, all arranged in series as shown in the drawing.

The coil box A may be of any ordinary construction for holding a coil 10 of a strip 11 of steel or the like, and permitting the 95 same to unwind for a continuous annealing; and the strip leveler B may include two sets of rolls 12 of any well known construction and operation, for flattening the sheet and removing uneven fullness or buckles which 100 may have been caused by reducing rolls or other apparatus used in producing the strip.

The spot welder C may include a set of electrodes 13 mounted in a frame 14 supported on a carriage 14' provided with wheels 15 riding on a track 16, together with gripping devices 14'', on the front and rear sides of the frame, for clamping and holding successive strips with their ends overlapped, in position between the electrodes for a spot welding operation while the carriage is traveling forward on the track.

The solution washer D may include strip supporting rolls 17 and transverse tubes 18 suitably apertured for spraying a hot soda 115 solution upon the strip, to remove grease and grit therefrom; and like tubes 18'' may also be provided for air drying the strip in rear of the cleaner.

The heating furnace E may include a cylindrical shell 20 mounted on supports 21 lined with a thick body of heat insulating material 22, within which is provided a lining of fire brick 23 or other refractory material, forming a support for electric resistors 24 and 24' 120 parallelly positioned above and below and forming between them a longitudinal heating chamber 25, in which are provided a series of transverse skids 26 for supporting a strip 11 as it is moved endwise through the chamber 125

from the entering slot 20' at its front end to the cooling duct F at its rear end.

- By these means, the strip may be heated directly by the action of the electric resistors, 5 in a uniform manner from end to end of the furnace, and the degree and continuity of heat can be readily controlled at all points in the heating chamber, by referring to the series of pyrometers 25'.  
 10 The cooling duct F may be a series of end connected iron tubes 27 and 27' extending rearward from the rear end of the furnace and the sections of the same may be surrounded by tanks or troughs 28 containing water 15 for cooling the conduit and the strip moving through the same.

The cooling troughs may be provided with a water inlet pipe 29, a water connecting pipe 29' and an overflow pipe 29'' so as to cause 20 a continuous flow of cooling water from the forward end toward the rear end of each trough.

The cleaning tank G may include an end closed trough 30 containing a weak solution 25 of sulphuric acid, with transverse skids 31 in its bottom for supporting the strip 11 and provided with rolls 32 in each end for guiding and holding the strip downward in the acid bath. A supporting roll 33 may be located at each end of the cleaning tank for 30 guiding the strip out of the cooling duct, into and out of the cleaning tank.

The washing tank H may include an end closed trough 34 containing water or other 35 washing liquid, with a guide roll 35 in each end and a supporting roll 36 at the rear end, for directing the strip through the water in the trough to wash from the same any acid or other coating which may be carried from 40 the cleaning tank.

The conveyer rolls I may include two stands of pinch rolls 38 arranged for drawing a strip through the apparatus and conveying it rearward to the double shear J, and between these rolls may be provided transverse 45 pipes 31' suitably apertured for hot air drying the strip.

The shear J is provided with a shearing die 39 on its front and rear sides, and a shearing punch 40 operating between them, for shearing the joint of two strips in front and in rear of their overlapped ends, so as to neatly disconnect them after the annealing process is completed.

The strip coiler K may be of any well known construction for winding the annealed strip 11' into a coil 10', and it is preferably provided with an independent motor 41 for this purpose.

In the operation of the apparatus, a strip sheet, which has been flattened by the leveler B, joined to another strip by spot welder C, and acted upon by the solution washer D, is moved continuously endwise through the 60 heating chamber 25 and the cooling duct F

wherein it is heated quickly and uniformly by the electric resistors to an annealing temperature, which temperature of the metal is maintained and continued only for the brief period necessary for a proper annealing of 70 the metal, which may not exceed one minute, whereupon it is promptly cooled quickly by the heat absorbing water surrounding the tubular duct. The strip is then cleared in the cleaning tank G and the washing tank H, 75 from any discoloration there may be on its surface.

In this manner a continuous quick annealing and pickling is accomplished, and the brief period during which the annealing temperature is maintained and continued, avoids the formation of a detrimental scale and prevents the production of an objectionable grain growth or "Stead's brittleness", so that the annealed strip thus produced is characterized by a uniformly fine grained structure and a highly ductile quality, which adapt it 80 for deep drawing operations.

By the improved apparatus strip sheets of different gauges and of more than ordinary 90 widths can be continuously annealed without developing any objectionable grain growth. In actual practice, any given portion of a strip sheet, one-sixteenth of an inch in thickness, may be heated to a temperature of 1400° 95 F., maintained at that temperature for about one-fourth of a minute, and then cooled to a nonoxidizing temperature, all within a period of about one and one-half minutes. This operation can be carried on continuously with 100 respect to all portions of each strip, and of successive strips which have been joined together, without stopping the movement of the strip which is passing through the heating chamber and the cooling duct. 105

The total length of the heating chamber and cooling duct of the apparatus may be about one hundred twenty-six feet, and the same may be operated so that a given portion of the strip sheet will pass through the 110 heating and cooling zone within a cycle of between three and four minutes, as diagrammatically illustrated in Figure 2 of the drawings.

Under these conditions, any given portion 115 of a strip sheet one-sixteenth of an inch in thickness, will be quickly heated by the direct action of the electric resistance, to annealing temperature, of say 1250° F., in a fraction less than one minute, and after being further 120 heated to a maximum temperature of say 1400° F., it is promptly cooled quickly to pass below the annealing temperature of say 1250° F., during the second minute of the cycle; so that the heat of the strip is only 125 maintained at an annealing temperature during a period of about one minute, thereby entirely avoiding, or reducing to a negligible minimum, the production of a grain growth in the body of the metal. 130

At the same time, the steel strip is quickly heated to a scaling temperature of say 1150° F., within a fraction less than one minute of the cycle, and after attaining the maximum temperature, is promptly and quickly cooled to below a scaling temperature, within a fraction more than the second minute of the cycle; so that a given portion of the strip is only maintained at a scaling temperature during a period of little more than one minute of the cycle, thereby avoiding the formation of a detrimental scale on the surface of the metal, and permitting the discoloration thereon to be readily removed by a weak cleaning solution, thereby producing a sheet with an even clean and clear surface.

We claim:

1. The method of annealing a steel strip which includes heating the strip quickly to annealing temperature, promptly cooling it quickly to avoid grain growth and scale and then cleaning the strip, all during a continuous endwise movement thereof.

2. The method of annealing a steel strip which includes heating the strip quickly to annealing temperature and promptly cooling it quickly to avoid grain growth and scale in a normal atmosphere, and then cleaning the strip, all during a continuous endwise movement thereof.

3. The method of annealing a steel strip which includes heating the strip quickly to annealing temperature and promptly cooling it quickly to avoid grain growth and scale in an atmospheric gas, then cleaning the strip and subsequently washing the same, all during a continuous endwise movement of the strip.

4. The method of annealing a steel strip which includes washing the same with a cleaning solution, then heating the strip quickly to annealing temperature in an atmospheric gas, then promptly cooling the strip quickly to avoid grain growth and scale, and then cleaning the same, all during a continuous endwise movement of the strip.

5. The method of annealing a steel strip which includes washing the strip with a cleaning solution, then heating the strip quickly to annealing temperature, and then promptly cooling the strip quickly to a non-oxidizing temperature to avoid grain growth and scale, all during a continuous endwise movement of the strip.

6. The method of annealing the body and cleaning the surface of a steel strip which includes heating the strip quickly to annealing temperature, then promptly cooling the strip quickly to a non-oxidizing temperature to avoid grain growth and scale, then cleaning the same, all during a continuous endwise movement of the strip.

7. The method of annealing the body and cleaning the surface of a steel strip which includes heating the strip quickly to annealing

temperature, then promptly cooling the strip quickly to a non-oxidizing temperature to avoid grain growth and scale, then cleaning the strip, and then washing the same, all during a continuous endwise movement of the strip.

8. The method of annealing a steel strip which includes uniformly heating the strip quickly throughout its width and thickness to annealing temperature, maintaining the same temperature only until the micro-structure of the metal is corrected, and then quickly cooling the strip to a non-oxidizing temperature to avoid grain growth, all during a continuous endwise movement of the strip.

9. The method of annealing a strip which includes uniformly heating the strip quickly throughout its width and thickness to annealing temperature in an atmospheric gas, maintaining the same annealing temperature only until the micro-structure of the metal is corrected, then quickly cooling the strip to a non-oxidizing temperature to avoid grain growth and scale, and then cleaning the strip to clear the surface thereof, all during a continuous endwise movement of the strip.

10. Apparatus for annealing steel strips, including a chamber for quickly heating the strip to annealing temperature, a tubular duct surrounded by heat absorbing liquid for promptly cooling the strip quickly from annealing temperature to avoid grain growth and scale, and a cleaning tank arranged in series for continuously annealing and cleaning the strip.

11. Apparatus for annealing steel strips, including a chamber for quickly heating the strip to annealing temperature, a tubular duct surrounded by heat absorbing liquid for promptly cooling the strip quickly from annealing temperature to avoid grain growth and scale, and a cleaning tank and a washing tank in series for continuously annealing, cleaning and washing the strip.

12. Apparatus for annealing steel strips, including a chamber for quickly heating the strip to annealing temperature, a tubular duct surrounded by heat absorbing liquid for quickly cooling the strip promptly from annealing temperature to avoid grain growth and scale, a cleaning tank, a washing tank and drying means, arranged in series for continuously annealing, cleaning, washing and drying the strip.

13. The method of annealing a steel strip which includes uniformly heating the strip quickly to annealing temperature, maintaining said temperature only until the micro-structure of the metal is corrected, and then quickly cooling the strip to avoid grain growth, all during a continuous endwise movement of the strip.

14. The method of annealing sheet steel which includes uniformly heating the steel quickly to annealing temperature, maintain-

ing said temperature only until the micro-  
structure of the steel is corrected, and then  
quickly cooling the steel to avoid grain  
growth.

5 15. The method of annealing a steel strip  
which includes heating the strip quickly to  
annealing temperature, promptly cooling it  
quickly to avoid grain growth and scale, and  
then cleaning the strip to remove discolora-  
10 tion therefrom, all during a continuous end-  
wise movement thereof.

16. The method of annealing sheet steel  
which includes heating the steel to annealing  
temperature, promptly cooling it quickly to  
15 avoid grain growth and scale, and then clean-  
ing the steel to remove discoloration there-  
from.

17. The method of annealing a steel strip  
which includes washing the same with a  
20 cleaning solution, then heating the strip

quickly to annealing temperature in an at-  
mospheric gas, then promptly cooling the  
strip quickly, and then cleaning the same,  
all during a continuous endwise movement of  
the strip.

25 18. The method of annealing a steel strip  
which includes uniformly heating the strip  
quickly by direct action of electric resistors  
to annealing temperature in an atmospheric  
gas, maintaining the same annealing tem-  
perature only until the microstructure of the  
metal is corrected, then quickly cooling the  
strip by indirect action of heat absorbing  
liquid, and then cleaning the strip to clear  
the surface of the same, all during a contin-  
uous endwise movement of the strip.

30 35 In testimony that we claim the above, we  
have hereunto subscribed our names.

HARRY M. NAUGLE.  
ARTHUR J. TOWNSEND.